

Patented Jan. 30, 1945

2,368,527

111

## UNITED STATES PATENT OFFICE

2,368,527

## TREATMENT OF CELLULOSIC PULP

Sidney M. Edelstein, Elizabeth, N. J.

No Drawing. Application September 10, 1942,  
Serial No. 457,889

7 Claims. (Cl. 260—212)

This invention relates to treated cellulosic pulp and the method of treatment. More particularly the invention relates to the making of a wood pulp of reduced and stabilized viscosity by treatment with hydrogen peroxide in proportion that is very small in relation to the amount of pulp treated and in conjunction with a metal of kind to be described.

The use of hydrogen peroxide to lower the viscosity of wood pulp has been known heretofore. It has been necessary, however, to use relatively large proportions of the peroxide.

I have now discovered that at least equal reduction in viscosity and better control of the operation may be effected by the use of much smaller proportions of peroxide than heretofore necessary provided the treatment with peroxide is made in the presence of iron, copper, aluminum, manganese, or like metal.

The invention comprises the method of treatment of pulp with the limited proportion of peroxide and the metal and also the resulting product. In the preferred embodiment, the invention comprises such treatment of pulp that has been previously reduced to a substantially pulverulent condition, effecting the treatment at a pH of approximately 6 to 8 and using the hydrogen peroxide on the anhydrous basis in proportion not substantially greater than 1% of the weight of the pulp and at a temperature between about 130° and the boiling point of the aqueous solution of the peroxide at the prevailing pressure, preferably between about 180° and 212° F. To avoid continuance of the reaction and objectionable uncontrolled variations of viscosity as the product stands, remaining peroxide is removed, as by centrifuging and rinsing, after the viscosity is lowered to the desired level.

Proceeding as described there is obtained the desired reduction in viscosity of the cellulose without other objectionable change. Thus the viscosity of alpha cellulose may be lowered to a tenth or less of the original, as from about 6,000 to 700 or even 100 or 200 centipoises as measured by test in sodium zincate solution. In this test there is formed a solution of the cellulose in standard concentration (5%) in a standard (10%) solution of sodium zincate and the viscosity is determined by the Stormer or an improved form of such viscosimeter.

The cellulose that has been so reduced in viscosity is suitable for use in making commercial solutions of cellulose in sodium zincate for application to textiles or the like and subsequent precipitation of a cellulose coating by the addi-

tion of sulfuric acid in amount to neutralize the alkalinity of the zincate solution. The treated pulp may also be used to make cellulose xanthate solutions for the manufacture of rayon or cellulose sheeting when low viscosity cellulose is desired. Also, the treated pulp is suitable for nitration in making pyroxylin for lacquer solutions.

As the cellulose used, there is employed wood pulp, cotton linters, rayon waste, or other pulp that is largely or practically entirely cellulose. Wood pulp and cotton are the preferred materials because of their relatively low cost and suitability. If wood pulp is used, the kind chosen is preferably a purified grade known as alpha cellulose. The cotton used is suitably that which has been purified by alkali digestion, to remove undesired ingredients.

In any case, the cellulose to be used should be in a state of fine subdivision and preferably substantially pulverulent so that it is reacted upon readily and substantially uniformly by the peroxide treating solution. A spun thread, for example, is not satisfactory. Neither is a fabric. While a usual loose pulp may be used under some circumstances, the cellulose for best results must be finely divided.

Such a substantially pulverulent cellulose is made by grinding or preferably cutting the selected cellulose to such fineness that it will pass largely through a 30-mesh screen or preferably through a 60-mesh screen. Actually I prefer to use cellulose which is predominantly 100-mesh or finer, difficulty having been found with material of the coarser meshes from lumping of the cellulose in the treating solution.

The moisture content during the comminuting of the cellulose may be that which is normally present in the air-dried material. When the moisture content is much higher, the cellulose may be made into a slurry and ground in a ball mill.

The viscosity reducing combination is hydrogen peroxide in contact with iron, copper, aluminum, or manganese, iron being particularly effective and constituting the preferred metal particularly when in the form of stainless steel. Stainless steel as the container for the reaction mixture is very satisfactory commercially in providing an adequate supply of iron and avoiding such an excess as might cause iron discoloration of the product.

The metal may be in massive form, as, for example, in the form of the container in which the reaction mixture is held or as a few added nails, or in the form of small pieces or fine powder pro-

vided there are no objections to the difficulty experienced in separating small pieces from the product or to some discoloration from the use of such pieces. In other words, the metal is present in elemental form.

The metal accelerates the reaction and makes unnecessary a large proportion of peroxide.

As the peroxide, only hydrogen peroxide is satisfactory.

The concentration of the peroxide solution which contacts the cellulose is very limited. There is thus provided better control of the reaction which, in the presence of the metal, is satisfactory in speed even at the low concentration of the peroxide. If a long time is to be allowed for the reaction, say a day or so, the concentration of the peroxide in the treating solution may be as low as 0.001%. Ordinarily there is used an aqueous solution of 0.001 to 0.1% concentration of hydrogen peroxide, all proportions of peroxide being given herein on the anhydrous basis unless specifically stated otherwise. Stronger solutions are not required or justified on the basis of cost. Ordinarily I use a solution of hydrogen peroxide of concentration about 0.003 to 0.03%.

It will be understood that the rest of the solution is ordinarily water and the concentrations given are the concentrations of hydrogen peroxide in the water solution which bathes the cellulose at the beginning of the treatment described.

It is very important to control the total amount of peroxide used in proportion to the cellulose being treated. Thus, it is necessary to use approximately 0.1 to 1 part of actual hydrogen peroxide for 100 parts of the cellulose. Ordinarily I start with a commercial 30% solution of hydrogen peroxide containing the conventional proportion of acid or other stabilizer for the hydrogen peroxide and add this to sufficient water at a temperature of around 210° F. to lower the proportion of peroxide to one of the concentrations given above. So much of the original 30% hydrogen peroxide is used as required to give about 0.1 to 1 part for 100 parts of the cellulose and to wet all the cellulose thoroughly. This amount is usually about 5 to 10 parts for each part of the cellulose. The cellulose is then introduced rapidly and vigorously stirred into the solution. The solution is heated approximately to the boiling point. The pH is established at 6 to 8. The cellulose, being added at ordinary temperatures, lowers somewhat the temperature, say to 180° F. or so, and the mixture is stirred at about this temperature for about an hour or two. The peroxide is then separated, as by centrifuging, so that the peroxide is removed from the remaining treated cellulose. Preferably the material is rinsed with cold water in the centrifuge till substantially free from peroxide, so that further uncontrolled reaction is avoided.

If the pH of the mixture as first made and before the warming to lower the viscosity of the cellulose is not within the range of approximately 6 to 8, a usual acid, alkali, or buffer as may be required is added to adjust the pH to that range. For a pH on either side of that range, there is a decreased rate of reaction of the hydrogen peroxide and metal combination in lowering the viscosity of the cellulose.

#### Example 1

Nine gallons of water are warmed to 210° F. in a stainless steel container provided with an agi-

tator. One pound of commercial 30% hydrogen peroxide is added to the liquid. Then 100 pounds of 92% alpha cellulose pulp which has been previously cut to 100-mesh fineness are added at one time. The mixture is agitated for about one hour, during which time the mixture slowly cools. The cellulose slurry is then discharged to a centrifuge and the cellulose is freed of the liquor as far as possible and finally washed with warm water. The pulp is then dried in an air drier or is used in the wet state for making solutions.

The initial viscosity of the cellulose before this treatment would be about 6,000 centipoises by the standard method described and after treatment about 1,000 centipoises.

#### Example 2

One hundred pounds of pulp as described in Example 1 are added to 100 gallons of water at 80° F. containing 3 pounds commercial (30%) hydrogen peroxide. This mixture is agitated for 24 hours in a wooden tank into which small pieces of iron have been introduced. After 24 hours the cellulose is separated from most of the remaining liquor in a filter press and thoroughly washed with warm water.

The viscosity change due to this treatment will be of the same order as in Example 1.

#### Example 3

The procedure of Example 1 to 2 is followed except that the prevailing pressure on the mixture is made superatmospheric, say 10 to 40 pounds gage, and the batch is heated to approximately the boiling point of the peroxide solution in an autoclave.

#### Example 4

The treated cellulose from any of the above treatments is substituted pound for pound in making cellulose zincate solutions in accordance with the description given in U. S. Patent No. 2,322,427, issued June 22, 1943, on an application filed August 19, 1941, for Cellulose product.

It will be understood that it is intended to cover all changes and modifications of the example of the invention herein chosen for the purpose of illustration which do not constitute departures from the spirit and scope of the invention.

What I claim is:

1. In the treatment of cellulosic pulp to lower the viscosity, the method which comprises forming a mixture including the pulp in pulverulent condition and a dilute aqueous solution of hydrogen peroxide, warming the mixture in contact with a metal in elemental form selected from the group consisting of iron, copper, aluminum, and manganese to a temperature between 130° F. and the boiling point of the aqueous solution under the prevailing pressure until the viscosity is reduced to the desired level, separating remaining hydrogen peroxide from the treated pulp, and then drying the product, the cellulosic pulp being of such fineness before treatment with the peroxide that the pulp will pass largely through a 30 mesh screen.

2. In making a cellulosic pulp of lowered viscosity, the method which comprises forming a mixture of wood pulp, of such fineness as to pass in predominating proportion through a 60 mesh screen, with a dilute aqueous solution of hydrogen peroxide at a pH of about 6 to 8 and warming the mixture in contact with a metal in elemental form selected from the group consisting of iron,

111

2,368,527

3

copper, aluminum, and manganese to effect the desired lowering of viscosity.

3. The method described in claim 2 the proportion of the hydrogen peroxide being not substantially in excess of 1 part on the anhydrous basis to 100 parts of the cellulosic pulp.

4. The method described in claim 2, the wood pulp before mixing with the hydrogen peroxide solution being previously reduced to substantially pulverulent condition causing the pulp to be so fine as to pass in predominating proportion through a 60 mesh screen and the aqueous solution of the peroxide being used in amount to wet thoroughly all of the cut wood pulp before the warming is undertaken.

5. The method described in claim 1, the metal used being iron.

6. The method described in claim 2, the metal used being in the form of stainless steel.

7. Treated cellulosic pulp comprising the product of the interaction of the pulp and hydrogen peroxide in contact with a metal in elemental form selected from the group consisting of iron, copper, aluminum, and manganese under conditions recited in claim 1, the said pulp being a powder of fineness to pass in predominating proportion through a 60 mesh screen and of such low viscosity that when dissolved in aqueous sodium zincate solution in the proportion of 5 parts of the pulp to 100 parts of the zincate solution, the viscosity of the resulting solution at 25° C. is 100 to 1500 centipoises.

SIDNEY M. EDELSTEIN.